

## UNITED STATES PATENT OFFICE.

JOHN WOOD LEADBEATER, OF DONCASTER, ENGLAND.

## PROCESS FOR MAKING DECOLORIZING CARBON FROM PEAT.

No Drawing.

Application filed May 12, 1919. Serial No. 296,665.

*To all whom it may concern:*

Be it known that I, JOHN Wood LEADBEATER, residing at Doncaster, in the county of York, England, have invented new and useful Improvements in Processes for Making Decolorizing Carbon from Peat, of which the following is a specification.

This invention relates to improvements in the means and method of obtaining carbon from peat,—in closed chambers,—for decolorizing purposes, such as, for example, say, for decolorizing sugar solutions, or edible, or vegetable, or mineral, or other oils, or paraffin wax and the like, and in apparatus for drying and carbonizing peat.

In this invention a dry mixture of dried peat alone and good ground caustic lime (unslackened ground lime) is employed. The lime being added to the peat helps to break up and disintegrate the fibres of the peat and a charcoal of low density and specific gravity is produced in a granular friable state due to the use of a dry mixture for distillation. The production of carbon by this process does not require grinding before further treatment and the production of volatile distillation products (oils, acetic acid, methyl alcohol, and the like) are in slight excess of the amount obtained by the distillation of peat alone.

According to this invention the peat is obtained in the usual and ordinary manner, and in its natural state contains more or less moisture. The percentage of the moisture varies according to the nature of the bog from which it is obtained. Before treating it for obtaining a decolorizing carbon from peat according to this invention the peat requires to be either air-dried in the usual manner, or dried in a furnace or retort, such as, say, an ordinary D-shaped coal gas retort, or any other suitable retort or oven, capable of being fixed in a framework, may be employed and heated to a suitable temperature depending on the moisture in the peat to be carbonized, or any other convenient mechanical means may be employed for drying purposes.

If the peat be dried in retorts or in a furnace the moisture should not be reduced beyond the percentage present in air-dried peat.

When the peat contains say from twenty-five to forty per cent of moisture, then a suitable temperature increasing from about five hundred and fifty to two thousand de-

grees Fahrenheit could be employed, but I would distinctly have it understood that the just named percentage and degrees, as well as any other percentages, degrees, or weights, may be varied or altered as circumstances require.

For drying the peat, other than by air, a furnace or oven or a retort, having trays therein for preventing the waste of the material operated upon, is provided with one or more exits for the gas and other products accumulating therein, and the said gas or products are conducted to a holder or other receptacle by a pipe, or pipes provided with one or more valves or stop cocks. The retort is made of metal or fireclay, or other suitable or refractory material and it is open at one or both of its ends, which end or ends is or are subsequently covered by one or two detachable doors made gas-tight by any convenient means, and retained in position by the bridge piece and screw, or by any other suitable means, such as are used in gas works for closing and sealing the ends of the retorts. If desired, though not necessarily so, a retort open at both ends may have, in the case of very long retorts, a transverse division piece at or about its centre.

The peat to be treated can be placed in an ordinary retort or oven for drying purposes, but preferably in the trays or receptacles, and after it has been ground it is necessary at the later stage to place it in trays or receptacles instead of being placed directly into the retort, so as to avoid the waste that would otherwise occur.

The peat after being dried is ground or crushed or finely divided for reducing it to a granular state or form and it is then laid in layers to form a bed. The layers of ground or crushed dried peat are each thoroughly mixed with a percentage of good ground caustic lime,—unslackened or quick lime,—say, in the proportion of, about, five pounds avoirdupois of lime to each one hundredweight of dried ground peat. The lime being added to the peat in a caustic state helps to break up and disintegrate the fibres of the peat.

After the peat and the just mentioned percentage of unslackened lime have been well mixed together in any suitable manner and by any ordinary means the dry mixture is placed in the trays. On the retort being heated to the required temperature,—say,

for example, increasing from five hundred and fifty to two thousand degrees Fahrenheit,—the carbonization is effected or aided by the action of the lime by disintegrating 5 the fibrous matters in the peat and there is a slightly increased yield of tar. Such carbonization is effected without access of air to the material in the retort. The resultant tar by-products are recovered by any ordinary 10 means and in the same manner as in coal gas manufacture, and the lime employed also slightly increases the yield of the by-products. From the resultant tar various light or heavy oils, acetic acid, 15 methyl alcohol, and the like may be distilled in the ordinary way.

After the above described process of carbonization has taken place the resultant residue will be in the form of powdered or 20 granular charcoal or carbon and therefore no grinding is required. The said resultant residue contains more or less percentage of ash or foreign and deleterious substances which vary according to the locality or 25 source from which the peat is obtained.

Some of the carbons made from peat have varying quantities of ash or foreign substances or impurities such as alumina or silica, or sand. For the purpose of removing 30 such impurities the carbon (obtained as above described from peat) is treated with hydrochloric acid, or sulphuric acid, or hydrofluoric acid, or any other acid or combination of acids. The quantities of such 35 acids, or combination of acids, vary according to the quantities of the impurities,—found by analysis,—that would interfere with or retard the decolorizing effect of the peat carbon.

40 When the quantity and nature of the impurities have been ascertained,—by analysis,—the residue from the just named carbonization is placed in a suitable lead lined vessel and boiled in water to which is added 45 and mixed,—say, for example,—hydrochloric, or sulphuric, or hydrofluoric acid of the ordinary commercial strength, or such other acid or acids as are or may be found requisite to treat and remove the ash or 50 foreign substances and impurities from the peat charcoal or carbon. If the ash or foreign substances or impurities amount to, say, about ten to fifteen per cent of the resultant residue then it is first treated with 55 about, say, a two per cent solution of hydrochloric or other acid. If after the boiling with the just named solution of hydrochloric acid there is still found,—by analysis,—any ash or foreign substances or impurities, such 60 as alumina, or silica, or sand, remaining in the resultant residue it may be found necessary to treat it with one or more other acids, which will vary according to the nature of the ash or foreign substances or impurities 65 remaining in the residue.

The mixture after being treated as above described is placed in an ordinary filter press and washed with pure water for removing the acid or acids before being again placed in the trays for drying purposes. 70 The trays and their contents are then inserted in the retort a second time for completing the carbonizing process and drying the resultant residue to the required degree of moisture.

After the residual carbon has been treated with the acid solution and before being placed in the retort or oven a second time there is added to and mixed or combined with the material, that is the acid washed residual carbon or charcoal obtained from the treatment of the peat, twenty-five to fifty per cent,—these quantities may be varied as circumstances require,—of fuller's earth, or hydrated silicate of aluminium, or kieselguhr, or diatomite, or other infusorial earth containing nearly pure silica.

Owing to the finely divided state of the decolorizing carbon obtained from peat by the said process, the particles of carbon are very liable to be carried through the filter and to pass into the syrup or oil being treated, thereby causing or producing a cloudiness in the latter. The addition of fuller's earth not only prevents this, but at the same time a better and more efficient decolourizer is obtained.

The material is then a second time placed in the above named retort or oven and heated or dried therein.

In practice it has been found difficult to get a single decolorizing agent to completely decolourize an oil, a certain portion being difficult to remove when a single agent has been used. Further, no single agent is equally efficient with all oils, due to the fact that the nature of the colouring matters in any oil is probably different from the colouring matters in another oil, and that one decolorizing agent is more efficient in withdrawing one colour than another. Thus fuller's earth seems to have little effect in removing the colouring matters present in sesame oil or ground nut oil while it produces a very marked effect in decolorizing 113 cotton seed oil, so that a mixture of agents, each removing different portions of the colouring matter of the oil is much more satisfactory than a single agent.

The function appears, from experiments made, to be possessed by the mixture of the decolorizing carbon,—produced from peat,—with fuller's earth with regard to cotton seed oil. The said decolorizing carbon taken alone has rather a less effect on cotton seed oil than on other oils, though this effect is considerable compared with that of ordinary animal charcoal.

Each of the said two agents,—the decolorizing carbon and the fuller's earth,—prob- 130

ably withdraws a different portion of the colouring matters present in the cotton seed oil for a combination of the two agents are much more effective than when either of 5 them are taken singly.

A decolorizing agent produced according to this invention is not merely a mixture of the said carbon and the fuller's earth in the proportions named, but such a mixture 10 which has afterwards been dried and heated. An additional effect is obtained by heating the two ingredients together whereby the decolorizing effect of the mixture thus treated is greater than the effect of an ordinary 15 untreated mechanical mixture of two ingredients.

What I claim is:—

The herein described method of preparing a material for decolorizing sugar solutions, and oil comprising drying finely divided peat, mixing the dried and finely divided peat with finely divided caustic lime, heating 20 said mixture to carbonize the peat therein, treating the residual carbon with an in-organic acid to remove ash and foreign sub-25 stances therefrom, combining the cleaned carbon with an infusorial earth, and finally heating and drying the mixed materials.

JOHN WOOD LEADBEATER.

Witnesses:—

W. FAIRBURN-HART,  
ALICE MARY TURNER.